

# UNITED STATES PATENT OFFICE.

JOHN T. HARROP, OF GARFIELD, NEW JERSEY.

## METHOD OF REPAIRING ASPHALT PAVEMENTS.

1,230,894.

Specification of Letters Patent. Patented June 26, 1917.

No Drawing.

Application filed May 23, 1916. Serial No. 99,314.

To all whom it may concern:

Be it known that I, JOHN T. HARROP, a citizen of the United States, and residing at Garfield, in the county of Bergen and 5 State of New Jersey, have invented certain new and useful Improvements in Methods of Repairing Asphalt Pavements, of which the following is a specification, such as will enable those skilled in the art to which it

10 appertains to make and use the same.

This invention relates to the art of repairing or restoring what are usually known as asphalt pavements, or pavements in which the top or wearing surface is of varying 15 thickness, and composed of asphalt, or a bituminous concrete, or a composition of variable sizes of stone, gravel, and sand, or like material, in combination with a bituminous binder, and the object of the invention 20 is to provide a method for the purpose set out whereby a worn down, broken, depressed or otherwise injured surface of a roadway or pavement of the class specified may be restored in an efficient manner and made 25 flush with the original surface and as strong and durable as said original or uninjured surface of said pavement or roadway; and with this and other objects in view the invention consists of an improved method of 30 repairing or restoring worn down places, depressions, breaks or holes in pavements of the class specified, no matter how large the worn down places, depressions, breaks or holes may be. Whenever the word depression 35 is used alone in the following specification, it will be understood to include worn down places, breaks, holes or other injuries of any kind to the surface of the pavement.

As is wellknown, pavements of the class 40 specified are usually laid on a base, of concrete, broken stone, gravel and sand, or similar material and this base may also contain a binder of bituminous material, but the character of the base, or the method of making it form no part of my invention.

In the practice of my invention, I preferably first thoroughly cleanse or clean the surface of the depression, hole or break in the wearing surface of the pavement, and 50 this may be done by sweeping or brushing, or by means of an air blast; and said depression after it has been cleaned in this manner may also be washed, if desired. The next step in the process is to impregnate or saturate the material in which the depression occurs, and the material immediately surrounding the depression, with a suitable

inflammable solvent such as gasoline or other similar highly inflammable petroleum product which tends to cut back and soften the 60 bituminous material in which the depression occurs. After the solvent has thoroughly impregnated the bituminous material it is ignited and allowed to burn for a period of time to thoroughly dry the base, and dry 65 out any moisture that may be therein and also in the surrounding or contiguous pavement, and to heat the base of the surrounding or contiguous pavement to a predetermined degree and to bring the surrounding 70 or contiguous pavement and the material in which the depression occurs to a plastic condition to receive the new or additional bituminous concrete or similar material used in repairing the injury to the pavement and 75 to form a flux and with which said material readily unites.

When the required temperature of the material in which the depression, break, or hole occurs, and the surrounding or contiguous material of the pavement is reached, and said material softened or made plastic to take the new material to be used in repairing the depression, the flames are extinguished by using a fireproof mat or in any other way, 80 and the depression is filled by first placing therein a layer of broken stone, slag, gravel or the like which is thoroughly compressed by tamping or rolling, after which bitumen heated to a temperature of approximately 90 three hundred and twenty-five degrees is poured over the said material, and covered with variable sizes of stone, gravel, slag, sand or like material and then tamped or rolled down hard to form a surface flush 95 with the surface of the old or original pavement. If the worn down pavement, depression, break or hole is of sufficient depth a layer of broken stone, gravel, sand and the like is first put in the depression, break or 100 hole and covered with asphalt or other bituminous binder, after which another layer of stone, gravel, sand or the like is placed on the asphalt or bituminous binder, and this is covered with another layer of asphalt 105 or bituminous material, and in this way there may be several layers of stone, slag, gravel, sand or the like and asphalt or bituminous material successively placed in the depression, break or hole, and whenever a 110 layer of stone, gravel, sand or the like is used it must be thoroughly tamped or rolled.

In preparing the worn down pavement, depression, break or hole in the first in-

stance, as herein set out, the surrounding or contiguous asphalt, or bituminous concrete, or similar material of the original pavement may be picked or roughened in any way to insure a more ready union therewith of the asphalt, bituminous binder, or bituminous concrete used in repairing the depression, break or hole.

With my improved method it is immaterial whether the surface of the asphalt, macadam or other pavement be worn down, broken or only depressed, in the latter case, however, the cleaning out of the depression will be carried out in the manner set forth, and said depression will be saturated or impregnated with a liquid petroleum product or other highly inflammable liquid which will be ignited and burned till the asphalt or other bituminous concrete or other material of the pavement in the depression and adjacent thereto is heated to a plastic condition, after which the said depression may be filled in with divided stone, gravel or the like to be tamped or rolled down and onto which will be poured liquid asphalt, bitumen, tar or any other suitable substance of this class which would operate as a binder, which substance will afterward be covered with sand, finely divided stone, screenings or like material which would then be tamped or rolled to form a firm hard surface.

It must also be understood that in repairing holes or breaks of any kind even where the surface of the pavement is removed, after the hole or break has been cleaned out and heated by burning a suitable inflammable liquid therein, the said hole, or break may be filled in with layers of broken stone, slag, gravel, sand or the like on which may be poured liquid asphalt, water gas tar or any like substance, which will operate as a binder, and this substance will then be covered by sand, finely divided stone, slag or the like, after which the surface of the filling will be tamped or rolled in the usual manner, or the depression, break or hole may be filled in with a hot or cold bituminous concrete which is raked into position, after which said bituminous concrete will be tamped or rolled to form a hard and dense finish, and in the use of a bituminous or similar concrete, as herein set out, either a hot or cold mix may be employed.

By means of my improved method worn down, broken, depressed or otherwise injured pavements of the class specified may be quickly and easily repaired, and at an expense comparatively small, and this may be done even in the winter-time and when the places to be repaired are frozen, if there is no frost in the concrete or other material

used for filling purposes, as the burning of the highly inflammable material in the 65 break or hole and on the surrounding pavement removes the frost therefrom and forms a flux with which said material readily unites.

I also desire it understood that wherever I have specified the use of bitumen or bituminous material as a binder that tar or similar material may be employed.

Having fully described my invention, what I claim as new and desire to secure by Letters Patent, is:—

1. The method of repairing depressions in asphalt or similar pavements which consists in first saturating or impregnating the material in which the depression occurs, with a suitable inflammable solvent, which cuts back and tends to soften said material, igniting and burning said solvent to render the material in which the depression occurs, plastic, and then filling in the depression 85 with a material containing a bituminous binder.

2. The method of repairing depressions in asphalt or similar pavements which consists in first saturating or impregnating the 90 material in which the depression occurs, with a highly inflammable petroleum product, which cuts back said material, igniting and burning said solvent to render the material in which the depression occurs 95 plastic, and then filling in the depression with a material containing a bituminous binder.

3. The method of repairing depressions in asphalt or similar pavements which consists in first saturating or impregnating the material in which the depression occurs, with a suitable inflammable solvent, which cuts back said material, igniting and burning said solvent to render the material plastic, and then filling in the depression with successive layers of broken stone, slag, gravel or the like and a bituminous binder.

4. The method of repairing depressions in asphalt or similar pavements which consists in first thoroughly cleaning the surface of the depression, saturating or impregnating the material, in which the depression occurs, with gasoline to cut back or soften the same, igniting and burning said gasoline 115 to render the material plastic, and then filling the depression with mineral material containing a bituminous binder.

In testimony that I claim the foregoing as my invention I have signed my name, in 120 presence of the subscribing witnesses, this 20th day of May, 1916.

JOHN T. HARROP.

Witnesses:

C. E. MULREANY,  
H. E. THOMPSON.